

## UNITED STATES PATENT OFFICE

2,306,576

## LINED CONTAINER

Albin H. Warth and William C. Rainer, Baltimore,  
Md., assignors to Crown Cork & Seal Company,  
Inc., Baltimore, Md., a corporation of New York

No Drawing. Application December 17, 1938,  
Serial No. 246,508

2 Claims. (Cl. 220—64)

The present invention is a composition for lining containers, and more particularly a composition of the wax type intended for lining sheet metal containers to be used in packaging liquids or other products, the taste of which is readily affected by wax.

The invention also relates to containers and to processes for preparing container-lining compositions.

Wax has long been recognized as a suitable material for lining containers of metal or other material, and it has been common practice to select a wax having properties suitable for the particular conditions under which the container is to be used; for example a wax having a sufficiently high melting point, and one which adheres to the metal or other material of the container throughout the range of temperature to which the container is subjected. In the packaging of beer, for instance, it is known that the beer must be pasteurized under a temperature as high as 145° F., and is frequently refrigerated as low as 40° F. Accordingly, a wax which adheres to the metal under these conditions is selected for the purpose of lining a container for beer. Again, the wax must have sufficient ductility to prevent breaking or cracking in the handling of the container, and must be sufficiently neutral in respect to the contents of the container so as not to impart objectionable taste.

The particular wax employed constitutes no part of the present invention, since the wax to be used involves merely a selection from known waxes of one having the quality desired for the particular conditions of use.

The present invention is based upon the discovery that waxes generally have a pronounced tendency to weaken or destroy the flavor of beverages, such as beer. We have found that these waxes have an affinity or "thirst" for the aromatic and flavoring constituents of beer, such as, for example, those principles or constituents which may be generally classified as ethers, esters and flavors derived from hops.

The invention is further based upon the discovery that it is possible to overcome this tendency by incorporating in the wax an agent which substantially satisfies or neutralizes this tendency of the wax to weaken or destroy the aromatic and flavoring constituents of beer. It has not been determined whether this tendency is due to the mere absorbency of wax or to some chemical reaction which occurs either during pasteurization or storage. But, in any event, we have found that it is possible to overcome this defect

by incorporating in the wax an agent which is substantially the equivalent of the aromatic or flavoring principle of beer which would otherwise be weakened or destroyed.

The invention is also based upon the discovery that it is possible to improve the film-forming characteristics of waxes of the general type above mentioned, and to overcome their tendency to produce a wavy or undulating surface which exhibits checks or lines marking the surface irregularities by including an agent which counteracts the tendency of the wax to form an irregular surface.

An object of the invention is to provide a wax lining composition so treated, as by the inclusion of an agent which reduces its adsorbent or flavor-weakening characteristic, that the contents of a lined container may be preserved for an indefinite period without an appreciable loss of flavor or color.

Another object of the invention is to provide a wax lining composition having the general characteristics which are required for the conditions under which the container is to be used and which will also form upon the container a uniform film having a smooth, even surface devoid of checks and surface irregularities.

In carrying out the invention, we select a wax or a combination of waxes which will provide, when hardened, a film which is closely adherent to sheet metal and is firm and adherent to the metal container wall under all conditions of use and is devoid of objectionable brittleness so that it will not break upon bending or denting of the container wall. The wax should also have a sufficiently high melting point so as to withstand the temperatures to which the contents of the container are subjected during pasteurization.

Any suitable wax may be employed; for example petroleum or petrolatum wax or a mixture of waxes, and in this connection may be used bleached beeswax (insect waxes), also refined ozokerite wax (earth waxes), as well as the waxes produced from petrolatum by the pressing and sweating, distillation, or selective solvent extraction processes employed in the manufacture of mineral oil waxes, particularly those of amorphous characteristics.

In the wax, we include an agent which will neutralize the tendency of the wax to adsorb, chemically react with, extract, or otherwise reduce the flavor of the particular material to be introduced into the container for which the wax is intended as a lining, and we prefer, as an active agent, one which has a definite flavor im-

parting characteristic more or less typical of the flavor of the liquid with which the container is to be filled.

For example, in the wax lining composition for a beer can, we introduce a certain amount of hops or hops flavor. Instead of, or in addition to hops, other flavoring constituents of beer may be included in the lining composition, such as malt flavor.

The hops may be introduced by plunging into the melted wax a fabric bag having a sufficient amount of hops to impart to the melted wax within a limited period of time an aroma of hops while the wax is heated. The aroma produced and which is noticeable when the wax is heated will indicate the degree to which the tendency of the wax to destroy the flavor of the beer has been overcome.

The following will indicate a typical procedure which has been found satisfactory.

A suitable amorphous wax of the type above mentioned, or a combination of waxes, is melted and thoroughly mixed, and brought to a temperature of substantially 190° F. before adding the hops. A mass of hops within a fabric bag is then lowered into the wax melt. The mixture should be kept at approximately 190° F. for a period of time, such as an hour or two, before removing the bag containing the hops. The period during which the hops is retained in the wax may be varied in accordance with the strength of the aroma desired, and this will vary with different waxes, depending upon their tendency to neutralize the beer flavor as may be readily determined.

The amount of hops to be introduced need not exceed approximately two and a half pounds to approximately eight hundred pounds of wax, although this amount may be varied, depending upon the strength of hops aroma and the wax permeation desired.

Generally, we have found that approximately three tenths of one percent of good quality of hops will be adequate.

As an alternative procedure, an amount of wax may be prepared which is very strongly permeated with hops as above or in the manner below disclosed, and this concentrated hops-containing wax may be introduced into the batch of melted wax so as to diffuse throughout the batch the desired amount of hops flavor.

If desired, the hops may be directly introduced into the batch and strained from the wax when the latter is poured into molds.

Instead of hops, we may use essence or oil of hops in small quantities, or Lupulin, i. e., a powder collected from the strobiles of hops.

The essence of hops may be imparted to the wax by allowing said wax to flow in a hop impregnated atmosphere for a time, or subjecting the wax in a thin layer to such atmosphere at normal temperature as for example, by treating of cans already lined with wax. The lined cans may be slowly conducted through a chamber, the atmosphere of which is suitably laden with hops aroma, and any desired pressure may be maintained in the chamber in order to insure a suitable impregnation of the wax with the hops aroma.

The hops aroma may, by these procedures, be increased as desired, even to the extent of making the aroma so distinguishable that it will positively impart to beer an added hops flavor.

In order that the wax may film suitably and provide a lining having a regular smooth and

unchecked surface devoid of irregularities, we preferably include in the same a check inhibiting agent or means to overcome differences in surface tension, namely, a high melting point amorphous wax derived either from a mineral or vegetable source which has been hydrogenated for the purpose of increasing the melting point and hardness; or treated by solvent extraction with filtering or centrifuging to obtain similar properties. We refer in particular to the I. G. waxes of commerce as sold by the General Dyestuff Corp., under the designation "I. G.-Waxes" as for example the I. G. waxes in the O. P. and A. D. forms. These waxes are represented as being free from impurities or unessential constituents, and have highly desirable amorphous characteristics.

In the use of these waxes in small amounts with the container lining wax we find that they may occasion a precipitation of small amount of substances when the melt is made; in which case it is desirable to filter off the precipitate as for example through cheese cloth. We prefer to use from seven tenths of one percent to two percent of IG-Wax OP, which has the following characteristics:

|               |     |         |
|---------------|-----|---------|
| Melting point | °F. | 221-226 |
| Acid value    |     | 10-15   |
| Ester value   |     | 110-125 |

30 Color Light yellow

The amount of the IG-Wax should be kept relatively low, due to the fact that it is extremely hard and tends to brittize the lining, enough being used only to avoid the checking heretofore encountered which we believe to be due to inequalities in surface tension and disclosed when the wax is hardened as by cooling.

The lining may be applied to a can or other metal container in any suitable manner, as by spraying or dipping, and the particular mode of application constitutes no part of the present invention.

Although we have referred particularly to the impregnation of wax lining compositions for beer containers, it will be understood that the invention is one of general application, and that wax intended for lining containers of liquids, beverages, or solids which tend to lose their flavor or aroma in the presence of wax may be similarly treated to reduce this tendency of the wax to extract the flavor or aroma. For example, a wax composition for lining containers for grape juice may be impregnated with oil of grape, and similarly lining compositions for containers for citric juices, such as orange or lemon juice, may be permeated with oil of lemon or oil of orange. The agent to be used will be one which will satisfy the thirst or adsorption characteristic of the wax for a particular flavor, and will not otherwise impart objectionable taste to the container contents.

It is to be understood that the inclusion in the wax of principles from hops, malt, and other flavors does not impair the physical and chemical characteristics of the wax for lining purposes, and after a batch of wax has been permeated with such principles, the wax may be hardened into blocks or other forms and retained in storage without appreciable loss of the desired principles.

We claim:

1. A container for beer and other food products having a wax lining, said lining adhering firmly to the wall of the container, being devoid

of brittleness and having a melting point above pasteurizing temperature, the said wax lining having incorporated therein not more than substantially 2% of a different and high melting point amorphous wax characterized by having a melting point of substantially between 221° to 226° F., an acid value of substantially between 10 and 15, and an ester value of substantially between 110 and 125 and being effective in the presence of the first wax to provide a lining having a regular, smooth and uncheckered surface.

2. A container for beer and other food products having a wax lining, said lining adhering firmly to the wall of the container, being devoid

of brittleness and having a melting point above pasteurizing temperature, the said wax lining having incorporated therein substantially .7 to 2% of a different and high melting point amorphous wax characterized by having a melting point of substantially between 221° to 226° F., an acid value of substantially between 10 and 15, and an ester value of substantially between 110 and 125 and being effective in the presence of the first wax to provide a lining having a regular, smooth and uncheckered surface.

ALBIN H. WARTH.

WILLIAM C. RAINER.